

May 12, 1942.

E. VAN DER PYL

2,282,912

## GRINDING WHEEL

Filed Sept. 11, 1939



Fig. 4

Inventor

EDWARD VAN DER PYL

Fig. 5

By George Crompton Jr.  
Attorney

## UNITED STATES PATENT OFFICE

2,282,912

## GRINDING WHEEL

Edward Van der Pyl, Holden, Mass., assignor to  
 Norton Company, Worcester, Mass., a corpora-  
 tion of Massachusetts

Application September 11, 1939, Serial No. 294,270

1 Claim. (Cl. 51—293)

The invention relates to grinding wheels and particularly diamond grinding wheels.

One object of the invention is to provide a facile method for attaching a diamond abrasive rim to a solid metal back. Another object of the invention is to make a grinding wheel which is metal throughout, that is consists of a metal back and an abrasive part which has abrasive grains bonded with metal without the necessity of pressing and sintering the backing but instead thereof using a cast or a machined metal backing. Another object of the invention is to form a firm union between a pressed and sintered metal bonded abrasive rim and a machined or cast metal backing. Other objects will be in part obvious or in part pointed out hereinafter.

The invention accordingly consists in the features of construction, combinations of elements, arrangements of parts, and in the several steps and relation and order of each of said steps to one or more of the others thereof, all as will be illustratively described herein and the scope of the application of which will be indicated in the following claim.

In the accompanying drawing showing one of many possible embodiments of the mechanical features of this invention,

Figure 1 is a cross sectional view through a mold in which is located the cast or machined backing and a mixture of abrasive and metal powders about to be pressed.

Figure 2 is a view the same as Figure 1 but showing the mold closed.

Figure 3 is an enlarged cross sectional view of that portion of the mold which contains the metal and abrasive powders prior to pressing.

Figure 4 is a view the same as Figure 3 but after the mold has been closed.

Figure 5 is a plan view of the backing, on the same scale as Figures 1 and 2, before it is placed in the mold.

Referring first to Figure 1 I provide an outer mold ring 10 and an inner mold block 11. In also provide a pressing ring 12. These parts the shapes of which are sufficiently indicated in Figures 1 and 2 constitute the mold. They may be located upon the platen 13 of a suitable hydraulic press and a top plunger, not shown, is used to close the mold with any desired pressure.

Located in the ring 10 and supporting the block 11 is a metal backing 15 that is going to form part of the finished article. This may be made in any suitable way but one of the objects of the invention is to dispense with the steps of pressing and sintering the metal backing or any

part thereof. That is to say it may be more convenient or economical to use a preformed backing 15. Such a backing can be cast, for example it can be made of cast steel. However I do not wish to limit myself to the use of castings since the backing might be machined from a blank and furthermore the backing might be formed by a forging process. Metals other than ferrous metals can be used such as copper, bronze, brass, aluminum. It is preferred, however, that the metal used as a backing have sufficient ductility or malleability so that it can be slightly deformed. Most of the ferrous metals have sufficient ductility or malleability excepting that gray cast iron is preferably not used. On the other hand wrought iron or malleable iron are readily usable carrying out my invention.

Referring now especially to Figures 3 and 5 I form undercut grooves 16 in the top surface of the backing 15 which in the illustrative embodiment has the form of a dish. This leaves annular ridges 17 which are preferably slightly undercut as shown. The annular ridges 17 have a dove-tailed shape in cross section. The grooves 16 may be cut with any suitable turning tool and in fact the grooving of the backing can well be effected in a lathe.

After placing the backing 15 inside the ring 10 and placing the block 11 upon the backing 15, as shown, I fill the annular space between them to a certain depth with an abrasive metal mixture in comminuted form. Preferably I use a mixture of diamond particles and copper and tin in powdered form as set forth in my Reissue Letters Patent No. 21,165. I prefer to use about 20% of tin and 80% of copper by weight and then form a total mixture of the powdered metals with diamond abrasive. I may provide diamonds to the extent of about 25% of the total mixture by volume but the proportion of abrasive can be widely varied. Using 50% of diamonds, or even more by volume, there is enough metal bond to make a strong article, while down to even 5% of diamonds will provide abrasive enough to do some cutting. Excellent results in actual practice, however, are achieved using 25% of diamonds by volume.

The metals should be finely divided but commercial powders are readily usable. The practical size of the diamonds will vary according to the type of finish that is desired, but I find excellent results in practice by the use of anywhere between 100 grit size up to 300 and even 400 grit size. Abrasive grit sizes are referred to which are measured by screens having that many

meshes to the linear inch given as the measure of the grit size.

I may also use other powdered metals and the invention is not to be deemed limited in any way to the particular metals specified. For example I may use any of the other mixtures specified in my Reissue Patent No. 21,165, namely copper and any of nickel, aluminum, manganese, or beryllium. Bonds made in accordance with my reissue Letters Patent are characterized by friability which has been found to be an excellent quality for metal bonds for diamond abrasive articles. In patent to Milligan No. 2,077,366 there are disclosed alloys of copper and aluminum, zinc and aluminum, silicon and nickel, silicon and iron, silicon and copper, and silicon and chromium and I may use any such alloys in powdered form or introduce the separate metals in powdered form into the mold. In my own prior Patent No. 2,077,345 I have disclosed a bond for diamond abrasive specifically consisting of 40 parts of aluminum and 60 parts of silicon and I may use this mixture.

With regard to whether to make an alloy of the two or more metals used and then powder the alloy or to use a mixture of powders each one being a powder of an elementary metal, practical considerations make the latter course preferable. The powders will sinter together forming an alloy readily enough if the melting points are not too far apart and it is easier to procure the elementary metal in powdered form. I may use electrolytic iron as disclosed in patent to Gauthier No. 1,625,463 or I may mix electrolytic iron with suitable proportions of carbon or any other ingredient to change the characteristics of the iron. On the other hand it is practical also to use finely divided steel or cast iron of a particular grade desired.

Having charged the mold with the desired mixture of diamond abrasive and powdered metal bond I place the pressure ring 12 in position as shown in Figure 1 and then "close the mold." This is done by bringing the upper platen of a hydraulic press down upon the ring 12 and forcing the top of it level with the ring 12 and the block 11. The effect of so doing is shown in Figures 2 and 4. The pressure acting through the partially plastic material 21 deforms the ridges 17, causing the area of their top surfaces to increase, increasing the overhang of the dovetails, and at the same time reducing them in height. At the same time, the pressure consolidates the loose mixture 21 into a rigid article which is locked to the backing 15.

After this operation I strip the now formed grinding wheel consisting of the backing 15 and the abrasive portion from the mold. This may be done in the usual manner and I provide tapped holes 22 in the block 11 for the insertion

of eye bolts to assist in the stripping. The abrasive portion is consolidated but greater strength can be imparted to it by a sintering operation. I now sinter the abrasive portion by placing the entire article in a furnace, preferably with hydrogen flame curtains, and raise the oven to a temperature slightly below the melting point of the metal which melts at the lowest temperature. In the case of the copper tin mixture mentioned first I may satisfactorily sinter at a temperature of 700° C. This sintering forms a homogeneous mass from the previously compressed powders and gives the metal bond the character of a true alloy.

It will be noted that the pressing operation greatly reduces the height of the ridges 17. Thereby but a small amount of total diamonds are embedded in the grooves 16. At the same time complementary dove-tails are formed in the grooves 16 to interlock with the dove-tailed annular ridges 17 to form a firm union between the abrasive portion and the backing 15. The article can be used for grinding right down to the tops of the ridges 17 and is not useless for grinding even after that, for, if a traverse is used, the abrasive dove-tailed annular ridges 22 will abrade and dove-tailed annular ridges 17 will readily wear down with the gradual wear of the abrasive. If desired the sintering may be done at the same time as the pressing and in such a case the press platens are heated and flames may be directed against the outer mold rim 10.

It will thus be seen that there has been provided by this invention a method and an article in which the various objects hereinabove set forth together with many thoroughly practical advantages are successfully achieved. As many possible embodiments may be made of the above invention and as many changes might be made in the embodiment above set forth, it is to be understood that all matter hereinbefore set forth, or shown in the accompanying drawing, is to be interpreted as illustrative and not in a limiting sense.

I claim:

Method of making a composite abrasive article which comprises forming annular dovetailed grooves with intervening annular dovetailed ridges in a ductile metal backing; placing the backing in a mold; filling the mold next to the grooves with a mixture of comminuted abrasive and comminuted metal; pressing the said mixture with a pressure sufficient to deform the ridges, causing the area of their top surfaces to increase, increasing the overhang of the dovetails, reducing them in height, thereby interlocking the pressed mixture with the backing; and then sintering the comminuted metal.

EDWARD VAN DER PYL.